

J. KILLEFER.  
Combined Share and Point.

No. 222,502.

Patented Dec. 9, 1879.



*Fig. 2.*



*Fig. 3.*



WITNESSES

Frank L. Ourand  
H. Aubrey Goulin

INVENTOR  
John Killefer  
Alexander Marion  
ATTORNEYS

# UNITED STATES PATENT OFFICE

JOHN KILLEFER, OF BLOOMINGDALE, MICHIGAN.

## IMPROVEMENT IN COMBINED SHARE AND POINT.

Specification forming part of Letters Patent No. **222,502**, dated December 9, 1879; application filed October 17, 1879.

*To all whom it may concern:*

Be it known that I, JOHN KILLEFER, of Bloomingdale, in the county of Van Buren, and in the State of Michigan, have invented certain new and useful Improvements in the Manufacture of Plowshares; and I do hereby declare that the following is a full, clear, and exact description thereof, reference being had to the accompanying drawings, and to the letters of reference marked thereon, making a part of this specification.

The nature of my invention relates to the manufacture of plowshares; and it consists in a combined plow share and point composed of a wrought-iron point and a cast-iron share made by heating the point to a welding-heat, placing it in a mold, and casting the share onto it, as will be hereinafter more fully set forth.

In the annexed drawings, Figure 1 is a view showing my improved plowshare. Figs. 2 and 3 show the flask or mold in which the share and point are united.

A represents the lower half of the flask or mold. B is the upper half of the same. C represents the plow-point, made of wrought-iron; and D is the space in the mold, made from any suitable pattern, into which the molten cast-iron is to be poured for forming the plowshare.

The wrought-iron point C is first heated to a proper degree for welding and then placed in the mold or flask in which the pattern has been molded. The mold or flask is then quickly closed and the molten cast-iron poured into the space D in contact with the heated wrought-iron point C, the molten cast-iron en-

tering the pores of the heated point, so as to make a perfect union between the two metals without any seam or division, except so far as the color of the metal will show.

I do not claim, broadly, the process of casting one kind of metal onto another kind of metal in a mold or flask, by heating one of the metals, for uniting the same, as I am aware that such process is not new.

I am also aware that a plowshare has been made of cast-iron with a steel point, by placing the steel point in the mold after said point has been properly prepared and tinned, and then casting the share onto it; and I do not claim such as my invention.

My combined plow share and point, as a new article of manufacture, consists of a wrought-iron point and a cast-iron share made by heating the point to a welding-heat, placing it in a mold, and then casting the share to it.

Having thus fully described my invention, what I claim as new, and desire to secure by Letters Patent, is—

As a new article of manufacture, a combined plow share and point consisting of a wrought-iron point and a cast-iron share made by heating the point to a welding-heat, placing it in a mold, and casting the share onto it, substantially as described.

In testimony that I claim the foregoing I have hereunto set my hand this 8th day of October, 1879.

JOHN KILLEFER.

Witnesses:

L. A. FOSTER,  
NAHUM GILBERT.